

6

July 20, 1937.

V. H. SANDERS

2,087,724

CARBON BRUSH AND METHOD OF MAKING

Filed Sept. 16, 1935

Fig. 1

408

3405  
X2034Fig. 2Fig. 3

## INVENTOR

Vernon H. Sanders

BY

Evans &amp; McCoy

ATTORNEYS

100  
101

## UNITED STATES PATENT OFFICE

2,087,724

## CARBON BRUSH AND METHOD OF MAKING

Vernon H. Sanders, St. Marys, Pa., assignor to  
Stackpole Carbon Company, St. Marys, Pa., a  
corporation of Pennsylvania

Application September 16, 1935, Serial No. 40,785

5 Claims. (Cl. 171—325)

This invention relates to molded brushes for  
motors or generators and similar electrical con-  
tact elements of the type known as carbon  
brushes, in which the conductive material con-  
5 sists mainly of carbon particles.

Objects of the invention are to increase the  
strength and durability of such brushes and also  
to lower the coefficient of friction of the brush  
so that objectionable chattering of the brushes  
10 on commutators is eliminated and the brushes  
ride more evenly on the rotating surface with  
which they engage.

In making the brush of the present invention,  
the finely divided conductive material consisting  
15 mainly of fine carbon particles is mixed with a  
suitable quantity of a resinous binding material  
preferably pitch or tar which may be coked or  
carbonized by heat treatment and the mixture is  
20 pulverized to a finely divided state. The pul-  
verized mixture is then molded under pressure in  
the form of blocks suitable for brushes, or may  
be molded in the form of elongated bars which  
25 may be cut to length to form a number of brushes,  
and after molding, the blocks or bars are baked  
at a temperature of from 1700° to 1800° F. for a  
time sufficient to coke or carbonize the binding  
material, with the result that the bars or blocks  
30 are hardened but are porous due to the coking or  
carbonization of the binder.

If desired the blocks may be further processed  
35 by subjecting them to a graphitizing heat which  
converts the carbon into the form of graphite.

Blocks prepared as above described have here-  
tofore been extensively used as brushes for  
35 motors or generators.

The brush of the present invention is, however,  
subjected to further treatment which increases  
its strength and durability and which also lowers  
its coefficient of friction so that the brush will  
40 operate more smoothly.

The carbon or graphite blocks formed as above  
described are placed in a conventional impreg-  
nating tank provided with means for applying  
pressure.

45 The blocks are placed in the impregnating tank  
and treated therein with a solution of resinous  
material which is capable of being hardened upon  
application of heat. The resinous material pref-  
erably used is a resinous material formed by the  
50 condensation of a mixture comprising a poly-  
hydric alcohol and a polybasic acid. This group  
of resins may be termed "glycerophthalate res-  
ins". The blocks are thoroughly impregnated  
55 with the solution by applying a suitable pressure  
in the impregnating tank and after impregnation

are dried to evaporate the solvent and then baked  
for from two to three hours in an oven heated  
from 350° to 700°. This heating polymerizes the  
resinous material which has been deposited in  
pores of the block upon evaporation of the sol-  
vent and forms a hard resinous coating on the  
walls of the pores interspersed throughout the  
body of each block, greatly increasing the  
strength of the blocks.

5 The glycerophthalate resin has the additional  
advantage of reducing the coefficient of friction  
of the brush, thereby eliminating chattering and  
insuring smoother operation.

The carbon particles may be in the form of  
graphite or amorphous carbon, and in the origi-  
15 nal baking the brushes may be subjected to suffi-  
cient heat to graphitize the block.

Referring to the accompanying drawing:

Fig. 1 is a perspective view showing a bar of  
the material from which the brushes are made; 20

Fig. 2 is a sectional view showing the tank in  
which the bars are impregnated;

Fig. 3 is a perspective view showing a com-  
pleted brush.

Carbon bars 1 such as shown in Fig. 1 are 25  
placed in a suitable impregnating tank 2 such as  
shown in Fig. 2 having a valve controlled vacuum  
pipe line 3, a valve controlled supply pipe line 4  
and a valve controlled drainage pipe line 5.  
After the tank 2 is charged with carbon bars 1, 30  
air is exhausted through the line 3, and solvent  
with the resinous material in solution is delivered  
into the tank through the line 5 under suitable  
pressure, and excess solvent being drained away  
35 through the line 5. Brushes such as the brush 6  
shown in Fig. 3 are formed from the impregnated  
carbon bars.

40 While the method of the present invention is  
ordinarily practiced in the manufacture of  
brushes from finely divided materials, it is obvious  
that the original molding and baking and the  
subsequent impregnation and baking may be per-  
formed at different times and places.

45 In one aspect thereof, the invention may be  
considered as a method of treating molded car-  
bon brushes to increase the strength and dur-  
ability thereof and improve the operating char-  
acteristics.

50 Furthermore, it is to be understood that the  
particular form of product shown and described,  
and the particular procedure set forth, are pre-  
sented for purposes of explanation and illustration  
and that various modifications of said prod-  
uct and procedure can be made without departing 55

from my invention as defined in the appended claims.

What I claim is:

1. An electrical contact element comprising a porous block composed of finely divided material consisting mainly of carbon held together by a carbonized binder and having the pores thereof partially filled with a polymerized resinous material.
2. An electrical contact element comprising a porous block composed of finely divided material consisting mainly of carbon held together by a carbonized binder and having the pores thereof partially filled with a polymerized glycero-phthalate resin.
3. The method of making electrical contact elements which consists of forming blocks of the desired shape by mixing finely divided material composed mainly of carbon with a glycero-phthalate resin, molding the mixture and subjecting the molded material to heat sufficient to carbonize the binder, impregnating the blocks so

formed with a solution of a resinous binding material, and heating the blocks to polymerize the glycero-phthalate resin.

4. The method of making electrical contact elements which consists of forming blocks of the desired shape by mixing finely divided material composed mainly of carbon with a resinous binding material, molding the mixture and subjecting the molded material to heat sufficient to carbonize the binder, impregnating the blocks so formed with a solution of a glycero-phthalate resin, and heating the blocks to polymerize the glycero-phthalate resin.

5. The method of treating carbon brushes of the type in which carbon particles are held together by a carbonized binder, which comprises impregnating a brush with a solution of a glycero-phthalate resin, evaporating the solvent and heating the brush to polymerize the glycero-phthalate resin.

VERNON H. SANDERS.